

## UNITED STATES PATENT OFFICE

2,219,411

## METHOD OF TREATING TIN CONTAINING MATERIALS

Fredrik Carlsson, Stockholm, Sweden, and  
Fredrick Trostler, London, EnglandNo Drawing. Application May 10, 1939, Serial No.  
272,920. In Norway May 16, 1938

7 Claims. (CL 75—85)

In the extraction of tin from low-grade (poor) ores, slags and the like, containing, for example, 40% or less of tin, it is already known to smelt the tin-containing material with approximately 5 50% of coke, with the addition of gypsum, in a shaft furnace, in the course of which there is driven off a (volatile) product very rich in tin. This method is, however, very expensive on account of the very great requirement of large-sized coke, particularly in the vicinity of the 10 mines, where suitable combustible material as a rule is obtainable only at a very high price. On the other hand, owing to the low content of tin, the transportation costs for the ore are too high 15 to permit transportation to the smelter without concentration. Besides, concentration frequently proves difficult and expensive owing to the complex composition of the ores.

The poorer tin ores that receive consideration 20 have a very different composition. The tin content, which usually occurs in the form of  $\text{SnO}_2$ , varies very much. The ores contain usually some pyrites, which by ordinary methods are removed by flotation, and also other sulphides. Sometimes 25 the content of pyrites may be considerable. The ores contain besides almost always varying amounts of silica and frequently iron oxide.

The present invention aims at a method, 30 whereby it is possible to volatilize the tin from the ore without previous extensive concentration, and afterwards recovering the same in the form of a compound rich in tin, and this without any addition or only with a small addition of carbonaceous combustible material.

In order to attain this the constituents of the 35 ore, and principally the pyrites, are utilized to produce the heat necessary for the process and simultaneously to change the tin into a volatile compound. In case the ore's content of sulphides 40 is too small, there will be added suitable sulphides, which usually can be obtained cheap at the mines, as well as free silicic acid (silica) if the ore contains too little of the same.

In carrying out the method of the invention, 45 the tin-containing material, with the addition if necessary of the required quantity of sulphide-containing fluxes (for example pyrites) and free silicic acid and if desired, other fluxes, is smelted in a shaft furnace which is provided with a closed charging arrangement, and in the lower 50 part of which air is blown in. The composition of the charge and the amount of the air blown in are adjusted in such a way that the greater portion of the tin will pass off with the smelting gases in the form of vaporous sulphide of tin and

the heat required for the process will be produced.

Where the composition of the tin ore from the mine varies, certain difficulties may be encountered in regulating the smelting process in such a 5 way that there will not occur now and then slight operating disturbances. In such cases it may be advantageous to add to the charge small quantities of a carbonaceous combustible material, for example 3-7% of coal or coke, whereby the necessary heat will be furnished for carrying through 10 of the entire process without disturbances.

If the charge contains sufficient quantities of pyrites, the course of the process will most likely 15 be as follows:

When the furnace charge, which preferably is preheated before charging, in the upper part of the furnace is heated by the gases coming from below to a temperature of 600-700° C., one sulphur atom of the pyrites commences to distill off. 20 If there is iron oxide in the charge, it will be converted to  $\text{FeS}$  with the formation of  $\text{SO}_2$ .

Somewhat deeper in the furnace, where the temperature is higher, the sulphides of the charge 25 will commence to react with the tin compound, whereby the tin is sulphidized, that is to say, it combines with sulphur and forms stannous sulphide and may be smaller quantities of stannic sulphide. If the temperature rises further, the sulphidizing becomes more lively and the tin sulphide vaporizes. At 1000-1050° C. the vaporization 30 is generally finished. The vaporized tin sulphide is condensed outside the furnace by cooling and is collected in dust chambers or other arrangements. If a portion of the tin sulphide is 35 oxidized by oxygen present in the furnace gases,  $\text{SnO}_2$  will be produced, which is carried along by the gases and is collected in the same way.

Of the other constituents of the charge  $\text{FeS}$  40 commences to melt at approximately 900°, drips down and is for the greater part oxidized just above the tuyères with the aid of the air blown in. At this place, from the quartz which has been charged in the shape of lumps there has been formed a skeleton, the so-called focus, as 45 soon as the furnace is in normal operation. By the oxidation there is formed under strong generation of heat  $\text{SO}_2$ , which rises, and  $\text{FeO}$ , which instantaneously combines with the  $\text{SiO}_2$  of the quartz. The other sulphides will also be partly 50 oxidized in a similar manner. The ferro-silicate formed combines with the slag-forming materials present and forms a slag, which flows out of the furnace together with the non-oxidized metallic sulphides (matte), for example to a fore 55

hearth, where slag and matte separate from each other.

The gases rising from the focus heat so strongly the charge lying above, that the reactions stated above can take place. The sulphur dioxide reacts partly with the metallic sulphides ( $FeS$ ) under formation of metallic oxides and elementary sulphur. If there is added to the charge a solid carbonaceous material, preferably in the form of small lumps then  $SO_2$  will also be reduced by the same. The thus generated sulphur vapor and the sulphuretted hydrogen, that may be formed with the aid of the moisture of the air, can also have a sulphidizing effect on the tin at the high temperature that is attained in the furnace.

As mentioned above, the sulphide of tin leaves the furnace in the form of vapor together with the other smelting-gases. In order to avoid condensation of the sulphide of tin and its settling in the upper part of the furnace, the furnace is run in such a way, that the outgoing gases have a high temperature, for example 800-1000° C. In order to attain this one must work with a lower column of the charge, and one can also preheat the charge or a portion of the same, before it is charged in the furnace.

In case not all of the tin should be sulphidized in the furnace and driven out, the slag that is flowing out of the furnace will contain tin principally in the form of oxide compounds. In that case one can, for example in the fore hearth, blow in  $H_2S$  in the molten mass (slag and matte) or also treat the charge, which still contains iron sulphides, with producer gas, coal dust or oil. Hereby the tin will be sulphidized and volatilized and can be collected jointly. However, it is desirous, of course, to regulate the composition of the charge and to carry on the operation in such a way, that by the temperature, that is effected in the focus, there is slagged the smallest possible amount of Sn.

If the stanniferous ore contains considerable amounts of iron oxide compounds, it is often advantageous to remove the same before the smelting. For that purpose the ore is finely divided and in an apparatus suitable therefor treated with a reducing gas, for example producer gas, at approximately 700-750° C., in such a way that the greater portion of the ferric oxide is changed into magnetite ( $Fe_3O_4$ ). By regulating of the temperature, the gas composition and the treatment period care is taken that the reduction is not carried too far, as there otherwise also would be produced  $FeO$ , which is unmagnetic. The material partly reduced in this way is subjected to a magnetic separator, during which the magnetite is removed.

The tin ore freed from a large portion of the iron oxide is briquetted together with an amount of quartz, pyrites and if required other fluxing agents, that is suitable for the subsequent smelting process, and the briquettes, after drying or hardening, are smelted in a shaft furnace.

The sulphide of tin produced by the present method is of a very high grade, and is remarkably suitable for manufacture of metallic tin or tin compounds.

Having now particularly described the nature of our invention and the manner of its operation what we claim is:

1. A process for the recovery of tin in the form of tin sulfide from tin containing ores, slags or the like, which comprises treating the tin containing raw material in the presence of a metal

sulfide and free silica in a shaft furnace provided with tuyères for the introduction of air blasts, while adjusting the composition of the charge and the quantity of air supplied to the furnace so as to convert the tin into tin sulfide and to produce a pyritic smelting in the furnace, said treatment being carried out in a shaft furnace having a closed charging arrangement to prevent oxidation of the tin sulfides formed by means of air admitted from above into the furnace and withdrawing from the furnace a gaseous product containing tin substantially in the form of tin sulfides.

2. A process for the recovery of tin in the form of tin sulfide from tin containing ores, slags or the like, which comprises smelting a charge of a tin bearing material containing a metal sulfide as well as free silica or other fluxes as required and a small quantity of a solid carbonaceous material in a shaft furnace having a closed charging arrangement and provided with tuyères for the introduction of air blasts, while adjusting the composition of the charge and the quantity of air supplied to the furnace so as to obtain a conversion of the tin into tin sulfide and to produce a pyritic smelting in the furnace, oxidation of the tin sulfides formed by means of air admitted from above into the furnace being prevented by said closed charging arrangement, and withdrawing from the furnace a gaseous product containing tin substantially in the form of tin sulfides.

3. A process for the recovery of tin in the form of tin sulfide from tin containing ores, slags or the like, which comprises mixing the tin containing raw material with pyrites and free silica, adding other fluxes and a small amount of a solid carbonaceous material, preheating said mixture, charging the preheated mixture in a shaft furnace having a closed charging arrangement and provided with tuyères for the introduction of air blasts, heating the charge while adjusting the supply of air into the furnace in such a way as to convert the tin into tin sulfide and to produce a pyritic smelting in the furnace, and withdrawing from the furnace a gaseous product containing tin substantially in the form of tin sulfides.

4. A process for the recovery of tin in the form of tin sulfides from tin containing ores, slags or the like, which comprises smelting a charge of tin bearing raw material containing pyrites and free silica in a shaft furnace having a closed charge arrangement and provided with tuyères for the introduction of air blasts, while adjusting the composition of the charge and the quantity of air supplied to the furnace so as to convert the tin into tin sulfide and produce a pyritic smelting in the furnace, withdrawing from the furnace a gaseous product containing the tin substance in the form of tin sulfides, the molten mass of slag and matte flowing out from the lower part of the furnace being treated with a sulphidizing gas, so as to convert to a sulfide the tin contained therein.

5. A process for recovery of tin in the form of tin sulfide from tin containing ores, slags or the like, which comprises crushing the tin containing raw material, subjecting said crushed material to a gas reduction in such a way that iron oxide present therein is reduced to magnetite, separating the magnetite from the other constituents, mixing said other constituents with pyrites, and quartz, and then briquetting the mixture, charging said mixture in a shaft furnace having a

closed charging arrangement and provided with tuyères for the production of air blasts, while adjusting the quantity of air introduced into the furnace so as to obtain a conversion of the tin into tin sulfide and to produce a pyritic smelting in the furnace, and withdrawing from the furnace a gaseous product containing tin substantially in the form of tin sulfides.

6. A process for recovery of tin in the form of tin sulfide from tin containing ores, slags or the like, which comprises crushing the tin containing raw material, subjecting said crushed material to a gas reduction in such a way that iron oxide present therein is reduced to magnetite, separating the magnetite from the other constituents, mixing said other constituents with pyrites and quartz, and then briquetting the mixture, charging said mixture in a shaft furnace having a closed charging arrangement and provided with tuyères for the introduction of air blasts, while adjusting the quantity of air intro-

duced into the furnace so as to obtain a conversion of the tin into tin sulfide and to produce a pyritic smelting in the furnace, and withdrawing from the furnace a gaseous product containing tin substantially in the form of tin sulfides.

5

7. A process for the recovery of tin in the form of tin sulfide from tin containing ores, slags or the like, which comprises mixing the tin containing raw material with pyrites and free silica, adding other fluxes, pre-heating said mixture, charging the pre-heated mixture in a shaft furnace having a closed charging arrangement and provided with tuyères for the introduction of air blasts, heating the charge while adjusting the supply of air into the furnace in such a way as to convert the tin into tin sulfide and to produce a pyritic melting in the furnace, and withdrawing from the furnace a gaseous product containing tin substantially in the form of tin sulfide.

10

15

FREDRIK CARLSSON. 20  
FREDRICK TROSTLER.